

May 7, 1940.

D. FINLAYSON ET AL

2,199,428

TEXTILE PRODUCT

Filed Aug. 20, 1937

FIG. 1



FIG. 2



FIG. 3



FIG. 4



FIG. 5



Inventors:

Donald Finlayson  
James F. Levers

J. Seltzer and B. Jefferson  
by  
Attorneys

## UNITED STATES PATENT OFFICE

2,199,428

## TEXTILE PRODUCT

Donald Finlayson and James Frederick Levers,  
Spondon, near Derby, England, assignors to  
Celanese Corporation of America, a corpora-  
tion of Delaware

Application August 20, 1937, Serial No. 160,066  
In Great Britain September 29, 1936

22 Claims. (Cl. 57—140)

This invention relates to improvements in textile products and is more particularly concerned with new composite yarns and with fabrics or other materials made of or containing such yarns.

5 It is well known that wool yarns are considerably more voluminous in character than cotton yarns and this is probably due at least in part to the fact that the fibres of cotton are considerably straighter than wool fibres and are comparatively 10 short in length so that it is necessary to insert a substantial amount of twist in a cotton yarn in order to obtain a coherent product, which reduces the voluminosity of such yarn. Moreover, 15 wool has a much greater elasticity both in the dry and wet state than has cotton.

For some purposes the voluminous and elastic 20 character of wool yarns presents considerable advantages and a great deal of research has been directed in recent years to the production of artificial 25 yarns which have the voluminous character of wool yarns. The results obtained, however, have not been entirely satisfactory since the products do not compare favourably with wool as regards their properties of voluminosity, elasticity 30 and non-crushability. For this reason many so-called artificial wools hitherto marketed have contained substantial proportions of natural wool, e. g. 50-75% of natural wool.

It has now been discovered that products which 35 have a very high degree of voluminosity and elasticity may be produced by associating a bundle, or yarn having at most only a low degree of twist, of crinkled filaments of cellulose acetate (as hereinafter referred to) with a yarn having a relatively high twist, i. e. a twist of the order of that necessary to impart to the yarn the capacity of shrinking on treatment with hot aqueous liquors. The yarn of high twist is hereinafter referred to as the basic yarn of the composite product. It is 40 important, in order to obtain the best results, that the yarn or bundle of crinkled filaments of cellulose acetate (hereinafter referred to as the voluminous component) should be present in preponderating proportions in the final product. Preferably, therefore, the basic yarn should 45 constitute as low a proportion as 30%, 20% or even less of the total denier of the composite product.

Crinkled filaments of cellulose acetate are obtained by subjecting bundles or yarns of cellulose 50 acetate filaments, especially such as comprise filaments of flat or nearly flat cross-section, to the action of hot or boiling water, or preferably hot or boiling dilute soap solutions. The flat type of filament is preferably produced by spinning a cellulose acetate solution in a normal way into an evaporative atmosphere but using a concentration 55 of cellulose acetate in the acetone or other volatile solvent lower than is customarily used to produce the bulbous type of filament. However, 60 the flat type of filament may also be produced

by spinning the cellulose acetate solution into an evaporative atmosphere which contains a high concentration of solvent for cellulose acetate near the spinning jets. Alternatively, or in addition, the spinning solution may contain paradichlorbenzene or other plasticising agent as described in British Patent No. 459,781. Other things being equal, a higher degree of crinkling, and therefore of voluminosity, is obtained with the higher filament deniers. The crinkling of the cellulose acetate filaments may be effected, for example, by treating such filaments, e. g. in the form of hanks of yarn, with hot aqueous liquors, and especially with hot dilute soap solutions, without tension so as to develop the crinkle in the filaments. The crinkle developed by the above processes is irregular in character.

Again, crinkle is imparted to cellulose acetate 20 filaments by processes such as those described in U. S. Patents Nos. 2,089,198 and 2,089,199 and British Patent No. 464,981. These processes consist, broadly, in imparting a twist to the yarns, setting the twist in the yarns, e. g. by the action of steam, and thereafter untwisting the yarns. Preferably the operation is effected with a false 25 twisting device. Such processes impart a spiral crinkle to the filaments. If desired the crinkling of the filaments may be accomplished by a combination of the two methods described above, e. g. a yarn or bundle of flat filaments of cellulose acetate may be subjected to one of the processes of U. S. Patents Nos. 2,089,198 and 2,089,199 and British Patent No. 464,981 and, either before or after such treatment, subjected to the action of 30 hot aqueous liquors.

The filaments in the voluminous component 35 may be continuous, as is normal in the production of cellulose acetate artificial silk, or may be discontinuous, provided that the length of the staple in the product is not so short as to necessitate a 40 relatively high degree of twist to produce a coherent product. A staple length of 5-8 or 10 inches or more may be used but preferably the staple is as long as possible, e. g. of the order of 18 inches.

The basic yarn may be of cellulose acetate or 45 any other suitable material for example of any other organic derivative of cellulose, or it may be of the regenerated cellulose type, e. g. viscose or cuprammonium silk or yarn obtained by complete saponification of cellulose acetate materials, or 50 it may be a partially saponified cellulose acetate material or may consist of a yarn of normal cellulose acetate which has been subjected to a process of acetylation as described, for example, in British Patents Nos. 448,816 and 448,917. Or, 55 again, the basic yarn may be of cotton, wool or natural silk. For reasons which are set out below it is especially advantageous to employ as the basic yarn a product of high tenacity, for example a cellulose acetate yarn which has been 60

stretched considerably so as to impart to it a high tenacity, or the product obtained by partial or complete saponification of such yarn. By employing a yarn of considerable strength as the 5 basic yarn it is possible to associate with it relatively large quantities of the voluminous component, and thus increase the total voluminosity of the product, whilst conserving the necessary strength for the product considered as a whole.

10 It is frequently advantageous, especially in the case of cellulose acetate materials and in the case when very high twists are being inserted, to insert the twist in the basic yarn of the composite product while the yarn is under the influence of 15 steam or hot water as described in U. S. Patents Nos. 2,088,628, 2,088,587 and 2,089,191.

The doubling twist used to associate the voluminous component with the basic yarn should not be so high as to reduce substantially the 20 voluminosity. As a result of the doubling operation the basic yarn either receives additional twist or has some twist removed therefrom depending on the relative directions of the twist in the basic yarn and of the doubling twist. For 25 this reason the twist in the basic yarn before the doubling operation should be either in excess of, or short of, that desired in the ultimate product. It is usually preferable to insert the doubling twist in the same direction as the original twist 30 in the basic yarn so that at no stage has the basic yarn a twist higher than that in the desired product. By this means the strength of the basic yarn is conserved. For example when an ultimate twist of 55 turns per inch in the basic 35 yarn of the composite product is desired, it is better to insert a twist of 50 turns per inch and then increase this to 55 by a doubling twist of 5 turns per inch in the same direction than to start with an original twist of 60 turns per inch and to 40 decrease this to 55 by a doubling twist of 5 turns per inch in the reverse direction.

Preferably the initial twist in the basic yarn and the doubling twist are so chosen that the basic yarn in the composite product is readily 45 capable of being shrunk by treatment with hot aqueous liquors.

As stated above it is of the greatest importance in order to obtain the best results that the voluminous component should be present in the 50 composite products of the present invention in preponderating proportion. The high proportion of voluminous component relative to basic yarn may be achieved, for example, by associating a voluminous component of relatively high denier 55 with a basic yarn of relatively low denier, the voluminous component and the basic yarn being fed at the same speed to the doubling device. Or alternatively, and this seems to be preferable 60 from the point of view of the voluminosity of the product, the voluminous component may be fed at a higher speed than the basic yarn to the doubling device, for example at a speed 5, 10, 50 or even 100% or more faster than that of the basic yarn. In this way the voluminous component 65 appears in the composite product as if it were more or less spiralled round the basic yarn, with the result that the latter may be more or less embedded in the composite product. As an example of the relative proportions of voluminous 70 component to basic yarn of a final total denier of 150-200 in the composite product, the basic yarn may have a denier of the order of 30-50. With such low proportions of basic yarn it is advantageous, as indicated above, that the basic yarn should be of relatively high tenacity.

In accordance with this invention a single basic yarn may be doubled with a single voluminous component but numerous other combinations fall within the scope of the invention. Thus two or more voluminous components may be 5 doubled with a single basic yarn, or two or more composite yarns, each containing one or more voluminous components doubled with a basic yarn, may be doubled together so as to make a product of greater total denier. Again, a voluminous component doubled with a basic yarn may be further doubled with an additional voluminous component, or composite yarns containing 10 one or more voluminous components doubled with a basic yarn may be doubled with each other and simultaneously with an additional basic 15 yarn or other desired component. In each doubling operation the speed of feeding the different yarns to the doubling device may be controlled in the manner already described so as to yield a 20 product of high voluminosity.

Preferably the composite products are subjected to a scour so as to shrink the basic yarn before associating the composite yarn in a fabric. By this means in the weaving or knitting of the 25 composite yarns into fabric not only does the presence of the basic yarn prevent undue extension of the voluminous component and thereby conserve the voluminous and elastic character of the composite yarn in the final product but, in 30 additional, the curl developed in the basic yarn as the result of the shrinking treatment helps to prevent slipping of the voluminous component along the basic yarn. However, the rough character of the basic yarn may be sufficient to prevent such slipping and the shrinking operation 35 may be applied to the materials, if desired, after fabric formation.

As indicated above, the initial twist in the basic yarn and the doubling twist are 40 preferably so chosen that the basic yarn in the composite product is readily capable of being shrunk by treatment with hot aqueous liquors. This is a characteristic of high twist "crêpe" yarn and the shrinkage in question may, therefore, be referred 45 to as a "crêpe shrinkage". The basic yarn, after it has been shrunk by treatment with hot aqueous liquors, is therefore referred to in the claims as a "crêpe-shrunk" yarn.

Examples of composite yarns according to the 50 invention will now be described with reference to Figs. 1-5 of the accompanying diagrammatic drawing.

In the drawing:

A is a 170 denier yarn of crinkled cellulose 55 acetate filaments substantially free from twist.

B is a 75 denier viscose crêpe yarn containing 40 turns per inch "S" twist.

C is a 75 denier viscose crêpe yarn containing 33 turns per inch "S" twist.

D is an 85 denier cellulose acetate crêpe yarn containing 100 turns per inch "S" twist prepared by a process in which the last part of the twist has been inserted while the thread is under the influence of steam. (See U. S. Patents Nos. 65 2,088,628, 2,088,587 and 2,089,191.)

E is a 34 denier natural silk crêpe yarn containing 74 turns per inch "S" twist.

F is a 75 denier viscose crêpe yarn containing 40 turns per inch "S" twist.

Referring to Fig. 1, one end of the yarn A is doubled with one end of the yarn B by means of 70 5 turns per inch "S" twist. If desired this construction can be modified by feeding the yarn A to the doubling device faster, e. g. 5% or 10% 75

faster, than the yarn B, and in this way the voluminosity of the product may be enhanced.

In Fig. 2, two ends of the yarn A are doubled with one end of the yarn C, the yarns A being fed to the doubling device 5% faster than the yarn C, i. e. each 100 units of length of the yarn C is doubled with 105 units of length of each of the yarns A. The doubling is effected by 12 turns per inch "S" twist.

10 The construction illustrated in Fig. 3 is similar to that shown in Fig. 2 except that one end of the yarn D is employed instead of the yarn C.

Fig. 4 illustrates a construction in which one end of the yarn E is doubled with one end of the 15 yarn A by means of 21 turns per inch "S" twist, the yarn A being fed to the doubling device 50% faster than the yarn E, i. e. so that 100 units of length of the yarn A are doubled with 150 units of length of the yarn E, and two composite yarns 20 thus produced are doubled together by means of a 12 turns per inch "Z" twist.

Referring to Fig. 5, two ends of the yarn F are doubled with one end of the yarn A by means of a 25 34 turns per inch "S" twist, the yarn A being fed to the doubling device at three times the speed of the yarns F, i. e. so that 100 units of length of each of the yarns F is doubled with 300 units of length of the yarn A, and two composite yarns thus produced are doubled together by means of a 30 12 turns per inch "Z" twist. The yarn produced in this way closely resembles a chenille yarn.

Having described our invention what we desire to secure by Letters Patent is:

1. A composite yarn resembling a wool yarn, 35 which comprises a yarn of crinkled cellulose acetate filaments which in the composite yarn has at most only a low degree of twist, doubled with a high twist yarn which in the composite yarn has a degree of twist such that it possesses the ability to shrink on treatment with hot aqueous liquors, the yarn of crinkled cellulose acetate filaments being present in substantially greater proportion than the said high twist yarn.

2. A composite yarn resembling a wool yarn, 45 which comprises a yarn of crinkled cellulose acetate filaments which in the composite yarn has at most only a low degree of twist, doubled with a high twist yarn which in the composite yarn has a degree of twist such that it possesses the ability to shrink on treatment with hot aqueous liquors, the yarn of crinkled cellulose acetate filaments being of substantially greater denier than the said high twist yarn.

3. A composite yarn resembling a wool yarn, 55 which comprises a length of a high twist yarn doubled with a greater length of a yarn of crinkled cellulose acetate filaments, the said yarn of crinkled cellulose acetate filaments having in the composite yarn at most only a low degree of twist, and the said high twist yarn having in the composite yarn a degree of twist such that it possesses the ability to shrink on treatment with hot aqueous liquors, the yarn of crinkled cellulose acetate filaments being in substantially greater 60 proportion than the said high twist yarn.

4. A composite yarn resembling a wool yarn, which comprises a length of a high twist yarn doubled with a greater length of a yarn of crinkled cellulose acetate filaments, the said yarn of 70 crinkled cellulose acetate filaments having in the composite yarn at most only a low degree of twist, the said high twist yarn having in the composite yarn a degree of twist such that it possesses the ability to shrink on treatment with hot aqueous liquors, and the said high twist yarn con-

stituting at most 30% of the total denier of the composite yarn.

5. A composite yarn resembling a wool yarn, 5 which comprises a high twist yarn doubled with a yarn of crinkled cellulose acetate filaments, the said yarn of crinkled cellulose acetate filaments having in the composite yarn at most only a low degree of twist, and the said high twist yarn having in the composite yarn a degree of twist such that it possesses the ability to shrink on treatment with hot aqueous liquors, the yarn of crinkled cellulose acetate filaments being in substantially greater proportion than the said high twist yarn.

6. A composite yarn resembling a wool yarn, 15 which comprises a yarn of crinkled cellulose acetate filaments doubled with a highly twisted yarn of high tensile strength, the said yarn of crinkled cellulose acetate filaments having in the composite yarn at most only a low degree of twist 20 and the said high twist yarn having in the composite yarn a degree of twist such that it possesses the ability to shrink on treatment with hot aqueous liquors, the yarn of crinkled cellulose acetate filaments being in substantially greater 25 proportion than the said high twist yarn.

7. A composite yarn resembling a wool yarn, which comprises a yarn of crinkled cellulose acetate filaments doubled with a highly twisted 30 yarn of high tensile strength, the said yarn of crinkled cellulose acetate filaments having in the composite yarn at most only a low degree of twist, the said high twist yarn having in the composite yarn a degree of twist such that it possesses the ability to shrink on treatment with hot aqueous 35 liquors, and the said high twist yarn constituting at most 30% of the total denier of the composite yarn.

8. A composite yarn resembling a wool yarn, 40 which comprises a yarn of cellulose acetate filaments which have been crinkled by treatment with a hot aqueous liquor, doubled with a high twist yarn which in the composite yarn has a degree of twist such that it possesses the ability to shrink on treatment with hot aqueous liquors, 45 the yarn of crinkled cellulose acetate filaments being present in substantially greater proportion than the said high twist yarn and having, in the composite product, at most only a low degree of twist. 50

9. A composite yarn resembling a wool yarn, which comprises a yarn of cellulose acetate filaments which have been crinkled by twisting the 55 yarn, setting the twist therein and thereafter removing at least part of the twist, doubled with a high twist yarn which in the composite yarn has a degree of twist such that it possesses the ability to shrink on treatment with hot aqueous liquors, the yarn of crinkled cellulose acetate filaments being present in substantially greater proportion 60 than the said high twist yarn and having in the composite product, at most only a low degree of twist.

10. A composite yarn resembling a wool yarn, which comprises a yarn of crinkled cellulose 65 acetate filaments which in the composite yarn has at most only a low degree of twist, doubled with a crêpe-shrunk high twist yarn, the yarn of crinkled cellulose acetate filaments being in substantially greater proportion than the said high 70 twist yarn.

11. A composite yarn resembling a wool yarn, which comprises a yarn of crinkled cellulose acetate filaments which in the composite yarn has at most only a low degree of twist doubled 75

with a crêpe-shrunk high twist yarn, the yarn of crinkled cellulose acetate filaments being of substantially greater denier than the said high twist yarn.

- 5 12. A composite yarn resembling a wool yarn, which comprises a length of a crêpe-shrunk high twist yarn doubled with a greater length of a yarn of crinkled cellulose acetate filaments which in the composite yarn has at most only a low degree 10 of twist, the yarn of crinkled cellulose acetate filaments being in substantially greater proportion than the said high twist yarn.
13. A composite yarn resembling a wool yarn, which comprises a yarn of crinkled cellulose acetate filaments which in the composite yarn has at most only a low degree of twist doubled with a crêpe-shrunk high twist yarn, the said high twist yarn constituting at most 30% of the 15 total denier of the composite yarn.
- 20 14. Process for the production of composite yarns resembling wool yarns, which comprises associating together at least two yarns, one of which is a yarn of crinkled cellulose acetate filaments and one of which is a high twist yarn, the 25 said yarn of crinkled cellulose acetate filaments being present in the final product in substantially greater proportion than the said high twist yarn and having in the final product at most only a low degree of twist, and the said high twist yarn 30 having in the final product a degree of twist such that it possesses the ability to shrink on treatment with hot aqueous liquors.
15. Process for the production of composite 35 yarns resembling wool yarns, which comprises doubling together at least two yarns, one of which is a yarn of crinkled cellulose acetate filaments and one of which is a high twist yarn, the said yarn of crinkled cellulose acetate filaments being of substantially greater denier than the said high 40 twist yarn and having in the final product at most only a low degree of twist, and the said high twist yarn having in the final product a degree of twist such that it possesses the ability to shrink on treatment with hot aqueous liquors.
- 45 16. Process for the production of composite yarns resembling wool yarns, which comprises feeding to a doubling device a yarn of crinkled cellulose acetate filaments and a high twist yarn, the former yarn being fed to the doubling device 50 at a speed greater than the latter yarn and the doubling twist being such that the said yarn of crinkled filaments in the final product has at most only a low degree of twist and the said high twist yarn has a degree of twist such that it possesses 55 the ability to shrink on treatment with hot aqueous liquors.
17. Process for the production of composite 60 yarns resembling wool yarns, which comprises feeding to a doubling device a yarn of crinkled cellulose acetate filaments and a high twist yarn, the former yarn being fed to the doubling device at a speed greater than the latter yarn and the doubling twist being in the same direction as the twist in the high twist yarn and being such that 65 the said yarn of crinkled filaments in the final product has at most only a low degree of twist and the said high twist yarn has a degree of twist such that it possesses the ability to shrink on treatment with hot aqueous liquors.
- 70 18. Process for the production of composite 75 yarns resembling wool yarns, which comprises doubling together at least two yarns, one of which

is a yarn of crinkled cellulose acetate filaments and one of which is a high twist yarn, in such proportions that the said high twist yarn constitutes at most 30% of the total denier of the product, and so that the said yarn of crinkled filaments possesses in the final product at most only a low degree of twist and the said high twist yarn possesses in the final product a degree of twist such that it possesses the ability to shrink on treatment with hot aqueous liquors. 10

19. Process for the production of composite 15 yarns resembling wool yarns, which comprises doubling together at least two yarns, one of which is a yarn of crinkled cellulose acetate filaments and one of which is a highly twisted yarn of high tensile strength, in such proportions that the said high twist yarn constitutes at most 30% of the total denier of the product, and so that the said yarn of crinkled filaments possesses in the final product at most only a low degree of 20 twist and the said high twist yarn possesses in the final product a degree of twist such that it possesses the ability to shrink on treatment with hot aqueous liquors.

20. Process for the production of composite 25 yarns resembling wool yarns, which comprises doubling together at least two yarns, one of which is a yarn of crinkled cellulose acetate filaments and one of which is a high twist yarn, so that the said yarn of crinkled filaments possesses in the final product at most only a low degree of twist and the said high twist yarn possesses in the final product a degree of twist such that it possesses the ability to shrink on treatment with hot aqueous liquors, and thereafter subjecting the 30 composite product to the action of hot aqueous liquors so as to effect shrinkage of such high twist yarn.

21. Process for the production of composite 35 yarns resembling wool yarns, which comprises doubling together at least two yarns, one of which is a yarn of flat cellulose acetate filaments which have been crinkled by treatment with a hot aqueous medium and one of which is a high twist 40 yarn, the said yarn of crinkled cellulose acetate filaments being present in substantially greater proportion than the said high twist yarn, and the doubling twist being such that the said yarn of crinkled filaments possesses in the final product at most only a low degree of twist and the said 45 high twist yarn possesses in the final product a degree of twist such that it possesses the ability to shrink on treatment with hot aqueous liquors.

22. Process for the production of composite 50 yarns resembling wool yarns, which comprises doubling together at least two yarns, one of which is a yarn of cellulose acetate filaments which have been crinkled by twisting the said 55 yarn, setting the twist, and removing at least part of the twist, and one of which is a high twist 60 yarn, the said yarn of crinkled cellulose acetate filaments being present in substantially greater proportion than the said high twist yarn, and the doubling twist being such that the said yarn of crinkled filaments possesses in the final product at 65 most only a low degree of twist and the said high twist yarn possesses in the final product a degree of twist such that it possesses the ability to shrink on treatment with hot aqueous liquors.